# EUROPEAN PATENT SPECIFICATION

(11) **EP 0 129 734 B1**
(45) Date of publication and mention of the grant of the patent: **31.01.1990**
(21) Application number: 84106102.1
(22) Date of filing: 29.05.1984
(51) Int. Cl.: C25B 11/04

(54) **Preparation and use of electrodes**
Herstellung und Anwendung von Elektroden
Préparation et utilisation d'électrodes

(30) Priority: 31.05.1983 US 499626
(43) Date of publication of application: 02.01.1985
(73) Proprietor: THE DOW CHEMICAL COMPANY, Midland Michigan 48640-1967 (US)
(72) Inventor: Beaver, R. Neal, Angleton Texas 77515 (US); Alexander, Lloyd E., Angleton Texas 77515 (US); Byrd, Carl E., Richwood Texas 77531 (US)
(74) Representative: Weickmann, Heinrich, Dipl.-Ing.

(56) References cited:
- EP-A- 0 046 449
- FR-A- 2 311 108
- US-A- 3 990 957
- US-A- 4 100 049

## Description

This invention pertains to an electrode, to a method for preparing this electrode and to its use in electrolytic cells, for example, brine electrolysis cells.

There are three general types of electrolytic cells used for the production of chlor-alkali: (1) the mercury cell, (2) the diaphragm cell, and (3) the membrane cell. The operation of each of these cells is discussed in Volume 1 of the Third Edition of the KIRK-OTHMER ENCYCLOPEDIA OF CHEMICAL TECHNOLOGY, page 799 et. seq. Other electrolytic cells which employ electrodes for electrolysis of aqueous solutions are the so- called "chlorate cells" which do not use a divider or separator between the cathodes and anodes. In the mercury cell, the alkali metal salt values produced by electrolyzing an alkali metal salt form an amalgam with the mercury; the amalgam, when reacted with water, produces NaOH and frees the mercury which can be recovered and cycled back for further use as a liquid cathode.

In many chlor-alkali electrolytic processes a brine solution (electrolyte) is electrolyzed by passing electric current therethrough in a cell having a diaphragm or a membrane positioned between the cathode and the anode. Chlorine is produced at the anode while sodium hydroxide (NaOH) and hydrogen (H₂) are formed at the cathode. Brine is fed continuously to the cells, while C1₂, NaOH and H₂ are continuously withdrawn from the cells.

The minimum voltage required to electrolyze an electrolyte into C1₂, NaOH and H₂ may be calculated using the thermodynamic data. However, in commercial practice, the theoretical amount of voltage is not achievable and higher voltages must be used to overcome the various resistances inherent in the various types of cells. To increase the efficiency of the operation of a diaphragm or a membrane cell one may attempt to reduce the overvoltages of the electrodes, to reduce the electrical resistance of the diaphragm or membrane, or reduce the electrical resistance of the brine being electrolyzed. The invention herein described results in an electrode particularly useful as a cathode in the electrolysis of brine; cathode overvoltage is substantially reduced, resulting in increased power efficiencies.

Because of the multi-million-ton quantity of alkali metal halides and water electrolyzed each year, even a reduction of as little as 0.05 volts in working voltage translates to very meaningful energy savings. Consequently, the industry has sought means to reduce the voltage requirement.

Throughout the development of chlor-alkali technology, various methods have been developed to reduce the cell voltage. Some practitioners have concentrated on reducing cell voltage by modifying the physical design of the electrolytic cell, while others have concentrated their efforts on reducing the overvoltage at the anode or the cathode. The present disclosure pertains, in part, to a novel process to make an electrode that is characterized by a significantly low overvoltage and to the use of these electrodes in electrolytic cells.

It has been disclosed that an electrode's overvoltage is a function of the current density and its composition (reference: PHYSICAL CHEMISTRY, 3rd ed., W. J. Moore, Prentice Hall (1962), pp. 406―408), where the current density refers to the amperage applied per unit of true surface area of an electrode and composition refers to the chemical and physical makeup of the electrode. Therefore, a process that will increase an electrode's surface area should decrease its overvoltage at a given apparent current density. It is also desirable to use a composition of matter that is a good electrocatalyst; this further reduces the overvoltage.

It is well known in the art to use plasma or flame spraying to coat an electrode with an electro- conductive metal. In U.S. Patent No. 1,263,959 it was taught that anodes may be coated by spraying fine nickel particles onto an anode, wherein the particles are rendered molten and impacted on the iron substrate by means of a blast.

Cathodes, also, have been coated with electroconductive metals. In U.S. Patent No. 3,992,278, cathodes were coated by plasma spraying or flame spraying an admixture of particulate cobalt and particulate zirconia. When these electrodes are used for the electrolysis of water or an aqueous alkali metal halide salt solution, they are said to give prolonged lowering of hydrogen overvoltage.

Various metals and combinations of metals have been used to coat electrodes by plasma or flame spraying: U.S. Patent No. 3,630,770 teaches the use of lanthanum boride; U.S. Patent No. 3,649,355 teaches the use of tungsten or tungsten alloy; U.S. Patent No. 3,788,968 teaches the use of titanium carbide or titanium nitride and at least one metal and/or metal oxide of the platinum group and a second oxide coating which is porous; U.S. Patent No. 3,945,907 teaches the use of rhenium; and U.S. Patent No. 3,974,058 teaches the use of cobalt as a coating with an overcoat of ruthenium.

It is, likewise, well known in the art to make porous electrode coatings by selective leaching. Coating an electrode with particulate nickel, then sintering the nickel as taught in U.S. Patent Nos. 2,928,783 and 2,969,315; electrodepositing an alloy onto a substrate then leaching out one component of the alloy as taught in U.S. Pat. No. 3,272,788; pressing or cementing two or more components together or onto an electrode substrate and then selectively leaching out one or more of the coating components as illustrated by U.S. Patent Nos. 3,316,159; 3,326,725; 3,427,204; 3,713,891 and 3,802,878.

It is also disclosed in the art to combine the steps of making electrodes by plasma- or flame-spraying followed by leaching. It is also disclosed to combine the steps of electroplating followed by leaching. Examples of known methods are illustrated in the following patents; U.S. Patent No. 3,219,730 teaches coating a substrate with a multiple oxide film coating then removing the substrate by leaching, thus forming an electrode; U.S. Patent No. 3,403,057 teaches flame or plasma spraying a Raney alloy onto a substrate followed by leaching aluminum out of the alloy thus leaving a porous electrode; U.S. Patent No. 3,492,720 teaches plasma spraying tungsten, titanium or alloys thereof along with aluminum, thorium and zirconium oxides onto a substrate. The substrate was subsequently removed, leaving a porous electrode.

U.S. Patent No. 3,497,425 teaches preparing porous electrodes by coating the substrate with a relatively insoluble metal followed by a coating of a more easily dissolvable metal. The teaching requires heat treating to cause inter-diffusion of the two coats, while optimum conditions require separate heat treatments for each coat. The dissolvable metal is subsequently leached out, leaving a porous electrode. U.S. Patent No. 3,618,136 teaches forming porous electrodes by coating a binary salt composition onto a substrate and leaching a soluble component from the system. The patent teaches that it is critical that the binary salt mixture is a eutectic composition and that optimum results are obtained when the same anions are used for both the active and the inactive salts, e.g. silver chloride - sodium chloride.

Netherlands Patent Application No. 75-07550 teaches the preparation of porous cathodes by applying to a substrate a coating of at least one non-noble metal from the group of nickel, cobalt, chromium, manganese and iron, alloyed with a secondary, less noble, sacrificial metal followed by removal of at least a part of this sacrificial metal. Specifically, the sacrificial metal is chosen from the group of zinc, aluminum, magnesium and tin. The sacrificial metal is removed by leaching with a lye solution or an acid solution.

Japanese Patent No. 31-6611 teaches forming a porous electrode by electroplating onto a substrate a nickel coating followed by a coating of zinc or some other soluble substance which is soluble in an alkaline solution. These coated electrodes are then either immersed in an alkaline solution or subjected to an electrochemical anodizing treatment to elute and remove zinc and other soluble substances, thus forming a porous electrode. Prior to immersion, a heat treatment of the coated electrode is required in some embodiments.

U.S. Patent No. 4,279,709 discloses a method for making electrodes including electrodes having reduced overvoltage by applying an admixture of particulate metal and a particulate inorganic compound pore-former and then leaching out the pore-former to form pores.

Electrodes of film-forming metal substrates, especially titanium, coated with oxides of Group VIII metals of the Periodic Table of The Elements have been taught, especially conjointly with other metal oxides, as being useful as anodes in electrolytic processes, such as in brine electrolysis. Ruthenium oxides, platinum oxides, and other oxides of the "platinum metal series", in association with various other metal oxides have received much acclaim as coatings for valve metal substrates (esp. Ti) for use as anodes. Patents relating to such anodes are, e.g. U.S. Patent Nos. 3,632,498 and 3,711,385. These coatings may be applied in several ways, for example, U.S. Patent No. 3,869,312 teaches that platinum group metal oxides, combined with film-forming metal oxides may be deposited on valve metal substrates by applying a mixture of thermally-decomposable compounds of platinum group metals and a thermally-decomposable organo-compound of a film-forming metal in an organic liquid vehicle which may also optionally contain a reducing agent, to a support member, drying the coating by evaporation of the organic vehicle, then heating the member in the range of 400-500°C to form metal oxides. Repeated coats are applied to increase the thickness of the coating. Also an overcoating of a film-forming metal oxide is applied. U.S. Patent 3,632,498 teaches that coatings of finely divided oxides of platinum group metals and film-forming metals may be produced by use of a plasma burner, by heating substrates which have been coated with thermally-decomposable compounds of platinum group metals and film-forming metals, by electrically depositing the metals in a galvanic bath followed by heating in air to form the oxide, among others.

Some further patents relating to electrodes having metal oxide surfaces are, e.g., U.S. Patent Nos. 3,616,445; 4,003,817; 4,072,585; 3,977,958; 4,061,549; 4,073,873; and 4,142,005.

The use of platinum group metal oxides, particularly ruthenium oxide, in active coatings for the evolution of hydrogen is also known (ref. Melendres, Carlos A., SPRING MEETING ELECTROCHEM. SOC., May 11-16,1975). Japanese patent publication no. 9130/65, application (OPI) nos. 131474/76 and 11178/77 refer to the use of a mixture of platinum group metal oxide(s) with another metal oxide as active cathode coatings. U.S. Patent No. 4,238,311 teaches that a cathode coating consisting of fine particles of platinum group metals and/or platinum group metal oxides in nickel is useful as a cathode coating.

In general, it is known by those skilled in the art that the use of oxides of platinum group metals as active catalysts for the evolution of hydrogen in modern electrolytic chlor-alkali cells employing permionic membranes is not useful because of extreme conditions of NaOH concentration and temperature now possible, wherein NaOH concentrations of 30% and temperatures exceeding 95° are not uncommon. Oxide coatings prepared according to the known art are found to decrepitate with use and fail by loss of adherence to the substrate, accompanied presumably by substantial reduction, in some cases, to base metals.

It is also well known to those practiced in the art that catalytic coatings consisting of metals with intrinsically low hydrogen overvoltage properties are subject in actual practice to loss of catalytic activity due to overplating with metallic contaminants, such as iron for example, which are commonly present in brine and water employed in the process of electrolysis. Consequently, active coatings found useful by those practiced in the art for evolution of hydrogen in modern electrolytic membrane chlor-alkali cells are limited to the type characterized by high surface area, or porous coatings, with compositions resistant to some degree to chemical attack at these conditions, e.g. nickel or various stainless steels.

In these cases, the full effect of the catalytic nature of intrinsically low hydrogen overvoltage catalysts are not realized in practice, since, as is well known to those practiced in the art, the performance of these essentially high surface area coatings degrades in time to a level characterized by the equivalent coating of the predominant metallic contaminant present in the brine or water employed in the electrolytic process, usually Fe. Consequently, the Tafel slope characterizing the electrolytic activity of the applied coating changes to essentially that of iron, with a resulting increase in hydrogen overvoltage, especially at higher current densities, 0.23 to 0.54 amp/cm² (1.5 to 3.5 amps/in²) and above, as are common in modern membrane chlor-alkali cells. In contrast, it is desirable to maintain the intrinsically low overvoltage properties of those materials which are known to be characterized by low Tafel slopes, i.e. platinum group metal oxides, particularly ruthenium oxide, during long-term operation in membrane chlor-alkali cells. It has now been discovered, among other things, that active coatings of oxides of ruthenium and secondary electrocatalytic metals when prepared according to the process of the invention, exhibit unexpected properties of low hydrogen overvoltage, physical stability, and long-term efficacy as cathodes in the electrolysis of brine at conditions of high NaOH concentrations, temperatures, and process pressures. It has also been discovered that the use of these electrodes in electrolytic processes wherein chlorine and caustic soda are produced at certain process conditions of temperature, NaOH concentration, pressure, etc., results in reduced energy requirements not otherwise attainable in practice.

The essential features of the electrode according to the invention are the subject-matter of present independent claim 1.

The invention also resides in a method for the production of an electrode, comprising a layer of an electro-conductive metal substrate and an electrocatalytically active coating deposited thereon, said coating being a heterogeneous mixture of metal oxides consisting of R_{U}0₂, NiO and metal oxides built from the metals of the electroconductive metal substrate or a previously applied coating, comprising the steps of applying a coating solution of metal oxide precursor compounds consisting of a Ru compound, a Ni compound and at least one chemically active agent capable of etching said substrate, thereby etching the surface of said substrate and/or any previously applied coating, concentrating the metal values of the precursor compounds and those etched from the substrate or previous coating by removing the volatiles from the so-coated substrate by heating and recoating them on the substrate or any previously applied coating and oxidizing the metal values by further heating the coated substrate in the presence of oxygen, air or an oxidizing agent.

Figure 1 illustrates graphically data from some of the tests described hereinafter.

The preferred electrically-conductive substrate may be any metal structure which retains its physical integrity during the preparation of the electrode. Metal laminates may be used, such as a ferrous metal coated with another metal, e.g., nickel or a film-forming metal (also known as valve metal). The substrate may be a ferrous metal, such as iron, steel, stainless steel or other metal alloys wherein the major component is iron. The substrate may also be a non-ferrous metal, such as a film-forming metal or a non- film-forming metal, e.g., Ni. Film-forming metals are well known in these relevant arts as including, notably, titanium, tantalum, zirconium, niobium, tungsten and alloys of these with each other and with minor amounts of other metals. Non-conductive substrates may be employed, especially if they are then coated with a conductive layer onto which the instant metal oxides are deposited.

The shape or configuration of the substrate used in the present coating process may be a flat sheet, curved surface, convoluted surface, punched plate, woven wire, expanded metal sheet, rod, tube, porous, non-porous, sintered, filamentary, regular, or irregular. The present novel coating process is not dependent on having a substrate of a particular shape, since the chemical and thermal steps involved are applicable to virtually any shape which could be useful as an electrode article. Many electrolytic cells contain foraminous (mesh) sheets or flat plate sheets; these are sometimes bent to form "pocket" electrodes with substantially parallel sides in a spaced-apart relationship.

The preferred substrate configuration comprises expanded mesh, punched plate, woven wire, sintered metal, plate, or sheet, with expanded mesh being one of the most preferred of the porous substrates.

The preferred composition of the substrate comprises nickel, iron, copper, steel, stainless steel, or ferrous metal laminated with nickel, with nickel being especially preferred. It will be understood that these substrates, onto which the metal oxide coatings are to be deposited, may themselves be supported or reinforced by an underlying substrate or member, especially where nickel, iron, or copper is carried by, or on, an underlying substrate or member. The substrate, onto which the metal oxide coating is to be deposited, may itself be an outer layer of a laminate or coated structure, and it may be, optionally, a non-conductive substrate onto which the metal oxide coating is deposited.

The soluble ruthenium compound may be the halide, sulphate, nitrate or other soluble salt or soluble compound of the metal and is preferably the halide salt, such as RuCI3. hydrate.

The secondary electrocatalytic metal oxide precursor of the present coating is at least one derived from a soluble compound of Ni.

The solution used in the present invention contains at least one chemically active agent capable of etching the substrate, and, in the case of second and later coatings, etching and solubilizing the most chemically-susceptible portions of the oxides previously formed, while also, preferably as the temperature is elevated, vaporizing, in many cases, from the heated mixture, along with volatilized anions or negative- valence radicals from the ruthenium oxide precursor and the Ni oxide precursor. The preferred chemically active etchants comprise most common acids, such as hydrochloric acid, sulphuric acid, nitric acid, phosphoric acid; also hydrazine hydrosulphate, and the like, with hydrochloric acid and hydrazine hydrosulphate being among the most preferred.

In general, the preferred method contemplated in the present invention comprises applying to the desired substrate a solution containing at least one ruthenium compound, at least one Ni compound, and a chemical etchant, preferably containing a volatile organic vehicle, such as isopropanol, leaving the etchant and the dissolved metal values; then heating the substrate to a temperature sufficient to concentrate the metal values, also substantially driving out the volatilized etchant along with the anions or negative- valence radicals released from the metal oxide precursors, and heating the substrate in the presence of oxygen or air to a temperature sufficient to thermally oxidize and convert the metals to metal oxides in-situ on the substrate. The steps may be repeated a plurality of times in order to attain the best full effect of the invention by increasing the thickness of the coating. Furthermore there is, at times, a benefit to be derived from laying down 2 or more layers of the metal oxide precursors between each thermal oxidation step.

In a particularly preferred embodiment an electrode material is prepared by applying a heterogeneous metal oxide coating, said heterogeneous metal oxide coating comprising nickel oxide and ruthenium oxide (optionally containing a modifier metal oxide, e.g., Zr0₂), into a nickel metal layer (which may be in the form of a nickel layer on an electroconductive substrate) by the process which comprises (a) applying to said nickel metal layer a coating solution comprising a nickel oxide precursor, a ruthenium oxide precursor, an optional modifier metal oxide precursor, and an etchant for dissolving the most soluble portions of the nickel metal surface, (b) heating to evaporate volatile portions of the coating solution, thereby concentrating and depositing the metal oxide precursors on the so-etched nickel metal surface, (c) heating in the presence of air or oxygen at a temperature between 300°C to 600°C for a time sufficient to oxidize the metals of the metal oxide precursors, and (d) cooling the so-prepared electrode material. Additional coatings may be applied in similar manner so as to increase the thickness of the so-produced heterogeneous metal oxide coating on the nickel metal surface, though the etchant for the second and later coating applications may beneficially be the same as, or different from, the etchant used in the initial coating application. There is thus prepared an electrode material comprising a nickel metal layer having tightly adhered thereto a heterogeneous metal oxide coating comprising nickel oxide and ruthenium oxide, optionally also containing a modifier metal oxide. The preferred optional modifier metal oxide is zirconium oxide. An economical form of the nickel metal layer is that of a nickel layer on a less expensive electro- conductive substrate, such as steel or iron alloys. Such electrode material is particularly useful as cathodes in chlor-alkali cells.

Ordinarily the temperatures at which thermal oxidation of the metals is achieved is somewhat dependent on the metals, but a temperature in the range of from 300° to 650°C, more or less, is generally effective. It is generally preferred that the thermal oxidation be performed at a temperature in the range of from 350° to 550°C.

The effect of the invention is to produce a substantially hard, adherent coating of heterogeneous oxides of the solubilized metals.

It is within the purview of the present inventive concept that the solubilization, reconcentration, and in-situ deposition of the solubilized metals, using chemical etching of the previously deposited layers and/or substrate produces an intimate mixture of oxides which are mutually stabilizing and electrocatalytically complementary.

The following examples illustrate particular embodiments, but the invention is not limited to the particular embodiments illustrated.

### Example 1

A solution was prepared which consisted of 1 part RuCL₃.3H₂0, 1 part NiC1₂-6H₂0, 3.3 parts H₂NNH₂.H₂SO₄ (hydrazine hydrosulphate), 5 parts H₂0, and 28 parts isopropanol. The solution was prepared by first mixing together all ingredients other than the isopropanol by stirring overnight, then adding the isopropanol and continuing to stir for approximately 6 hours.

A cathode was prepared which was constructed of a 40% expanded mesh of nickel. The cathode was first sandblasted, then etched in 1:1 HCI. It was subsequently rinsed, dipped in isopropanol and air dried. The cathode was coated by dipping it into the coating solution, allowing it to air dry, then baking it in an oven at 375°C for 20 minutes. In the same manner, a total of 6 coats were applied. The cathode was immersed in a heated bath containing 35% NaOH at a temperature of 90°C. A current was applied and potential measurements were taken using a standard Calomel Reference Electrode (SCE) and a Luggin probe. The cathode potential was measured at -1145 millivolts vs. SCE at a current density of 2 amps per square inch (0.31 amps per cm²). The cathode was assembled in a laboratory membrane chlorine cell and operated at 90°C, producing C1₂ at the anode and H₂ at the cathode, at 31-33% NaOH concentration, operating at 0.31 amp/cm² (2 amp/in²) current density. The potential of the cathode was monitored and averaged per week. The results are shown in Table I.

### Example 2

A solution was prepared which consisted of 1 part R_{U}C1₃-3H₂0, 1 part NiC1₂-6H₂0, and 3.3 parts concentrated HCI. It was allowed to mix overnight. Subsequently, 33 parts isopropanol were added and mixing continued 2 hours. A cathode was prepared in accordance with the procedure of Example 1. The cathode was then coated in the same manner as Example 1 except baking was carried out at a temperature of 495°-500°C. Ten coats were applied. The cathode potential was measured as in Example 1. The potential was -1135 millivolts vs. SCE. The cathode was assembled in a laboratory cell containing a commercially available NAFION^{*} polymer (^{*}a tradename of E. I. duPont de Nemours) membrane. The cell was operated at 90°C, 31-33% NaOH, and 0.31 amp/cm² (2 amp/in²) current density. The potential of the cathode was monitored and averaged per week. The results are shown in Table I.

### Example 3

A solution was prepared which consisted of 3 parts RuCL₃.3H₂0, 3 parts NiCl₂·6H₂O, 1 part ZrC1₄, 5 parts concentrated HCI, and 42 parts isopropanol. The solution was allowed to mix 2 hours. The cathode was then coated in the same manner as Example 1 except baking was carried out at a temperature of 495°-500°C. Eight coats were applied. A ninth coat was applied and the electrode was baked for 30 minutes at a temperature of 470°-480°C. The potential of the cathode was measured as in Example 1. The potential was -1146 millivolts vs. SCE. The cathode was assembled in a laboratory membrane chlorine cell containing a commercially available membrane, as in Example 2. The cell was operated at 90°C, 31-33% NaOH, and 0.31 amp/cm² (2 amp/in²) current density. The potential of the cathode was monitored and averaged per week. The results are shown in Table I.

### Example 4

A cathode was prepared as in the previous examples, then dipped in a solution containing 1 gram of tetraisopropyl titanate in 100 ml of isopropanol. The cathode was then baked at a temperature of 475°-500°C for 10 minutes. Three coats were applied. A solution was prepared as in Example 2. The cathode was dipped in the solution, air dried, and baked at a temperature of 475°-500°C. Six coats were applied. The potential of the cathode was measured as in the previous examples. The potential was -1154 millivolts vs. SCE. The cathode was assembled in a laboratory membrane chlorine cell containing a commercially available membrane, as in Example 2. The cell was operated at 90°C, 31-33% NaOH, and 0.31 amp/cm² (2 amp/in²) current density. The potential of the cathode was monitored and averaged per week. The results are shown in Table I and also in Figure 1.

### Example 5 (Comparative Example)

A 40% expanded mesh electrode of steel was prepared, but not coated, and assembled as the cathode in a laboratory cell as in Example 2-5, using the same type membrane. The potential of the cathode was monitored and averaged per week. The results are shown in Table I.

### Example 6 (Comparative Example)

A 40% expanded mesh electrode of nickel was prepared, but not coated, and assembled as the cathode in a laboratory cell as in Examples 2-5, using the same type membrane. The potential of the cathode was monitored and averaged per week. The results are shown in Table I and also in Figure 1.

### Example 7

The cells of Examples 2―6 were operated at 90°C, 31-33% NaOH, and 0.31 amp/cm² (2 amp/in²) current density while maintaining atmospheric pressures in the anolyte and catholyte compartments of the cell. Sodium chloride brine and water were fed to the anolyte and catholyte compartments, respectively, in order to maintain anolyte concentrations in the range 180-200 grams per liter NaCI and 31-33% NaOH. Internal mixing of the cells was accomplished by natural gas lift due to evolution of hydrogen gas at the cathode and chlorine gas at the anode. Data including mass and energy balances were collected periodically over the period of operation of the cells and energy requirements for the production of NaOH were calculated. The results are shown in Table 2.

### Example 8

In a large scale test, two series of pressure membrane chlorine cells were constructed. The construction and design of the cells were identical except that the series identified as Series 1 had nickel- wall cathode compartment and nickel electrodes installed in the catholyte compartment of the cells, while the series identified as Series 2 was constructed of steel-wall cathode compartment and steel cathodes. The electrodes of Series 1 were coated according to the process of the invention, while those of Series 2 were uncoated. Both series were erected with a commercially available cation exchange membrane, as in Example 2. The two series were operated simultaneously at 90°C, 0.31 amp/cm² (2 amp/in²) current density, and 31 to 33% sodium hydroxide in the catholyte chamber. The series were operated at pressures of 101,325 to 202,650 Pa (1 to 2 atmospheres) while recirculating the anolyte and the catholyte through the cells using centrifugal pumps. The ratio of the catholyte flow to the anolyte flow was maintained at a value greater than 1. Energy and mass balance data were collected and average performance data were calculated over a period of 45 days. The results clearly show that the energy savings attained with the use of the electrodes of the present invention (Series 1) averaged greater than a 5% reduction in energy, compared with Series 2.

It is within the purview of the present invention to employ the present novel electrodes at temperatures encountered in cells operated at superatmospheric pressures, as well as at atmospheric or subatmospheric pressures. The electrodes are especially suitable for operation in the elevated temperature range of from 85° to 105°C. Pressures at around 101,325 Pa (1 atm.), more or less, are ordinarily used in chlor-alkali cells, though pressures up to about 303,975 Pa (3 atm.) or more may be used.

The electrodes of the present invention are useful in cells wherein circulation within each electrolyte compartment is created by the gas-lift (displacement) action of gaseous products produced therein, though in some cells, such as in electrolyte series flow from cell-to-cell, another pumping means may be provided to supplement, or substitute for, the gas-lift action. We find it advisable, in some cases, to maintain the ratio of the volume of catholyte pumped to that of the anolyte volume pumped, at a ratio greater than unity.

The electrodes of this invention are useful in chlor-alkali electrolytic cells in which the anolyte has, or is adjusted to have, a pH in the range of from 1 to 5, such as when an acid, e.g. HCI, is added to the anolyte.

## Claims

1. An electrode for use in an electrochemical cell, comprising a layer of an electro-conductive metal substrate and an electrocatalytically active coating deposited thereon, characterized by the feature that said coating is a heterogeneous mixture of metal oxides consisting of R_{U}0₂, NiO and metal oxides built from the metals of the electro-conductive metal substrate or a previously applied coating, which have been solubilized by etching during the process of the coating of the electro-conductive metal substrate.

2. The electrode of claim 1, characterized in that the electro-conductive metal substrate is nickel.

3. The electrode of claim 1 to 2, characterized in that the electro-conductive metal substrate has a layer of nickel between it and the heterogeneous metal oxide coating.

4. A method for the production of an electrode according to claims 1-3, comprising a layer of an electro-conductive metal substrate and an electrocatalytically active coating deposited thereon, said coating being a heterogeneous mixture of metal oxides consisting of Ru0₂, NiO and metal oxides built from the metals of the electro-conductive metal substrate or a previously applied coating, comprising the steps of applying a coating solution of metal oxide precursor compounds consisting of a Ru compound, a Ni compound and at least one chemically active agent capable of etching said substrate, thereby etching the surface of said substrate and/or any previously applied coating, concentrating the metal values of the precursor compounds and those etched from the substrate or previous coating by removing the volatiles from the so-coated substrate by heating and recoating them on the substrate or any previously applied coating and oxidizing the metal values by further heating the coated substrate in the presence of oxygen, air or an oxidizing agent.

5. The method of claim 4, characterized in that the metal oxide precursor compounds are selected from metal chlorides, nitrates, sulphates and phosphates.

6. The method of claim 4, characterized in that the surface is etched with hydrochloric acid, sulphuric acid, nitric acid, phosphoric acid and/or hydrazine hydrosulphate.

7. The method of claim 4, characterized in that the coating procedure is repeated at least once.

8. The method of claim 4, characterized in that the temperature at which the oxidation of the metal values is carried out is in the range of from 300°C to 600°C and wherein the heating of the substrate takes place for a period of time of from 5 to 60 minutes.

9. Use of the electrode of one of the claims 1 to 3 as a low hydrogen overvoltage cathode in a chlor- alkali-electrolytic cell.

## Patentansprüche

1. Elektrode zur Verwendung in einer elektrochemischen Zelle mit einer Schicht eines elektrisch-leitenden Metallsubstrats und einer darauf befindlichen elektrokatalytisch aktiven Beschichtung, dadurch gekennzeichnet, daß die Beschichtung eine heterogene Mischung von Metalloxiden ist, bestehend aus Ru0₂, NiO und Metalloxiden aus den Metallen des elektrish-leitfähigen Metallsubstrats oder einer vorher applizierten Beschichtung, die durch Ätzen während des Verfahrens der Beschichtung des elektrishleitenden Metallsubstrats solubilisiert worden sind.

2. Elektrode nach Anspruch 1, dadurch gekennzeichnet, daß das elektrisch-leitende Metallsubstrat Nickel ist.

3. Elektrode nach Anspruch 1 oder 2, dadurch gekennzeichnet, daß sich zwischen dem elektrisch-leitenden Metallsubstrat und der heterogenen Metalloxidbeschichtung eine Nickelschicht befindet.

4. Verfahren zur Herstellung einer Elektrode nach einem der Ansprüche 1 bis 3 mit einer Schicht eines elektrisch-leitenden Metallsubstrats und einer darauf befindlichen elektrokatalytisch aktiven Beschichtung, wobei die Beschichtung eine heterogene Mischung von Metalloxiden ist, bestehend aus R_{U}0₂, NiO und Metalloxiden aus den Metallen des elektrisch-leitenden Metallsubstrats oder einer vorher applizierten Beschichtung, das die Stufen umfaßt: Applizieren einer Beschichtungslösung von Metalloxid-Vorläuferverbindungen bestehend aus einer Ruthenium-verbindung, einer Nickelverbindung und mindestens einem chemisch aktiven Mittel, das zum Ätzen des Substrats fähig ist, wodurch die Oberfläche des Substrats und/ oder eine vorher applizierte Beschichtung geätzt wird, Konzentrieren der Metallwerte der Vorläuferverbindungen und derjenigen, die aus dem Substrat oder der vorher applizierten Beschichtung abgeätzt wurden, durch Entfernen der flüchtigen Anteile aus dem so beschichteten Substrat durch Erhitzen und Wiederbeschichten des Substrats oder einer vorher applizierten Beschichtung mit ihnen und Oxidieren der Metallwerte durch weiteres Erhitzen des beschichteten Substrates in Gegenwart von Sauerstoff, Luft oder einem Oxidationsmittel.

5. Verfahren nach Anspruch 4, dadurch gekennzeichnet, daß die Metalloxid-Vorläuferverbindungen ausgewählt sind aus Metallchloriden, Nitraten, Sulfaten und Phosphaten.

6. Verfahren nach Anspruch 4, dadurch gekennzeichnet, daß die Oberfläche mit Chlorwasserstoffsäure, Schwefelsäure, Salpetersäure, Phosphorsäure und/oder Hydrazinhydrosulfat geätzt wird.

7. Verfahren nach Anspruch 4, dadurch gekennzeichnet, daß das Beschichtungsverfahren mindestens einmal wiederholt wird.

8. Verfahren nach Anspruch 4, dadurch gekennzeichnet, daß die Temperatur, bei der die Oxidation der Metallwerte durchgeführt wird, im Bereich von 300°C bis 600°C liegt, und das Erhitzen des Substrates während einer Zeitdauer von 5 bis 60 min stattfindet.

9. Verwendung der Elektrode nach einem der Ansprüche 1 bis 3 als Kathode mit geringer Wasserstoffüberspannung in einer Chloralkali-Elektrolysezelle.

## Revendications

1. Electrode pour utilisation dans une cellule électrochimique, constituée, d'une couche d'un substrat de métal électro-conducteur et d'un revêtement électrocatalytiquement actif déposé sur ce substrat, caractérisée par le fait que ledit revêtement est un mélange hétérogène d'oxydes métalliques comprenant Ru0₂, NiO et des oxydes métalliques composés à partir des métaux du substrat métallique électroconducteur ou d'un revêtement antérieurement appliqué, métaux qui ont été solubilisés par attaque chimique au cours du processus de revêtement du substrat de métal électro-conducteur.

2. Electrodé selon la revendication 1, caractérisé en ce que le substrat de métal électro-conducteur est le nickel.

3. Electrode selon la revendication 1 ou 2, caractérisée en ce que le substrat de métal électro- conducteur comporte une couche de nickel entre lui et le revêtement d'oxyde métallique hétérogène.

4. Procédé de production d'une électrode, selon les revendications 1-3, constituée d'une couche d'un substrat de métal électro-conducteur et d'un revêtement électrocatalytiquement actif, déposé sur élle ledit revêtement étant un mélange hétérogène d'oxydes métalliques comprenant Ru0₂, NiO et des oxydes métalliques provenant des métaux du substrat de métal électro-conducteur ou d'un revêtement antérieurement appliqué, procédé comportant les étapes consistant à appliquer une solution de revêtement, constituée de composés précurseurs d'oxydes métalliques comprenant un composé de Ru, un composé de Ni et au moins un agent chimiquement actif capable d'attaquer chimiquement ledit substrat, de façon à attaquer la surface dudit substrat et/ou tout revêtement antérieurement appliqué, à concentrer les métaux des composés précurseurs, et les métaux obtenus par attaque du substrat ou du revêtement antérieur, en éliminant par chauffage les produits volatils du substrat ainsi revêtu, puis à en revêtir à nouveau le substrat, ou tout revêtement antérieurement appliqué, et à oxyder les métaux en continuant à chauffer le substrat revêtu en présence d'oxygène, d'air ou d'un agent oxydant.

5. Procédé selon la revendication 4, caractérisé en ce que l'on choisit les composés précurseurs des oxydes métalliques parmi les chlorures, les nitrates, les sulfates et les phosphates des métaux.

6. Procédé selon la revendication 4, caractérisé en ce que l'on attaque chimiquement la surface avec de l'acide chlorydrique, de l'acide sulfurique, de l'acide nitrique, de l'acide phosphorique, et/ou de l'hydro- sulfate d'hydrazine.

7. Procédé selon la revendication 4, caractérisé en ce que l'on répète au moins une fois la procédure de revêtement.

8. Procédé selon la revendication 4, caractérisé en ce que la température à laquelle l'oxydation des métaux s'effectue se trouve dans l'intervalle allant de 300°C à 600°C et en ce que le chauffage du substrat s'effectue pendant une période de temps allant de 5 à 60 minutes.

9. Utilisation de l'électrode de l'une des revendications 1 à 3, en tant que cathode à faible potentiel hydrogène dans une cellule électrolytique chlore-hydroxyde alcalin.
